

ADDED

Patented Mar. 25, 1930

1,752,232

## UNITED STATES PATENT OFFICE

EDWIN D. CODDINGTON, OF MILWAUKEE, AND ERNEST A. KERLER, OF WEST ALLIS, WISCONSIN; ROE R. BLACK, OF PITTSFIELD, MASSACHUSETTS; AND HARVEY S. OWEN, OF MILWAUKEE, WISCONSIN, ASSIGNORS TO E. D. CODDINGTON MANUFACTURING COMPANY, OF NORTH MILWAUKEE, WISCONSIN, A CORPORATION OF WISCONSIN

## CEDAR PLASTER

No Drawing.

Application filed February 23, 1929. Serial No. 342,295.

The present invention relates to an improved wall surface or the like which has the inherent structural properties and advantages of a plaster and which embodies and gradually emits into the surrounding atmosphere the characteristic natural aroma and fragrance of cedar wood. The invention also contemplates the plaster composition which is used in forming such a wall surface, the formula of ingredients used in compounding the plaster, and the prepared mixture of essential ingredients which is furnished to the trade.

The efficiency and acceptability of natural cedar wood as an aromatic wall surfacing material, usually as an agent for protecting clothing and other articles and particularly for protecting against moths, has been long recognized and is exemplified by the extensive use of the wood for chests, closet linings, and the like. It is a particular object of the invention to provide a wall surface or the like which emits the true aroma of cedar wood, unaccompanied by any substantially sensible modifying odor or aroma, with a potency and permanence comparable to that of the wood itself, yet which is in every sense a plaster. The cedar plaster of the present invention is a substantially perfect substitute for natural cedar wood in the matter of emitting the fragrance and aroma of cedar, and also in its moth-proofing properties. Additionally, the product, being a plaster, offers certain important advantages which are not possessed by cedar wood.

It is an object of the invention to provide a plaster which brings to the user all of the benefits of cedar wood at a cost considerably less than the cost of cedar wood; which furnishes such benefits without the accompanying disadvantages of cedar wood; and which possesses certain important advantages over cedar wood such as ease of application, particularly in odd shaped and difficultly accessible places, freedom from joints, a surface which is hard, smooth and easily cleaned, and fire-proof and water-proof characteristics.

It is a further object of the invention to provide a formula for compounding a plas-

ter having the properties and characteristics above described, which formula is of such nature that a preparation containing all of the essential ingredients in proper proportion and intimate admixture can be made up in advance of the use of the material for plastering and will be stable during the ordinary course of manufacture, shipment, storage and use. The invention also specifically contemplates the particular composition of the specific plaster disclosed herein which has been used commercially with notably good results.

The aroma or persistent characteristic odor of red cedar is due to the volatile oil present in the wood. This oil occurs in the wood in amounts ranging from 1% to 2% in average cedar woods and from 2% to 4% in the red wood or pure heart wood of red cedar. It is the aroma arising from this volatile oil in the wood which has a protective effect for clothing and other articles. The oil can be extracted from the wood by appropriate processes as, for instance, by distillation of cedar wood sawdust or shavings. This extracted or recovered cedar wood oil embodies the aromatic principle of the cedar wood and is the ingredient of cedar wood which is responsible for its characteristic fragrance and aroma and its moth-proofing properties.

Cedar wood oil is present in the plaster of this invention, and it is the sole aroma emitting or insect repelling ingredient of the plaster. We have found that appropriate incorporation of this single aroma yielding ingredient into a plaster provides a wall surface which is substantially identical with natural cedar wood in the matter of giving out the fragrance and aroma of cedar into the surrounding air. No added insecticide or other ingredient is used which destroys, disguises or substantially modifies the natural cedar fragrance of the plaster imparted to it by the incorporated cedar wood oil. The present plaster product provides the characteristic aroma of cedar, the pleasing fragrance of the natural wood, and the insect repellent value of true cedar linings, all substantially indistinguishable from the corresponding characteristics of the natural wood.

It is this substantial duplication of the characteristics, benefits and advantages of true cedar wood in a plaster that is an important object of the invention.

As stated above, cedar wood oil is the active aroma yielding ingredient of the present cedar plaster. The use of this particular ingredient and the use of this ingredient alone as the active aroma yielding constituent, or at least unaccompanied by any other ingredient which destroys or sensibly modifies its own true cedar wood odor, is essential to the invention. No other ingredient satisfies the requirements of the invention; no other ingredient provides the true natural fragrance of cedar in the plaster. For example, cedar leaf oil is entirely unacceptable and is directly at variance with the concept of this invention. Cedar leaf oil is an entirely different product from cedar wood oil. It is derived from the leaf portion of the cedar tree and has an unattractive smell which is totally different from the fragrance of cedar wood. The term cedar wood oil is used herein to designate the oil, extract or essence of cedar wood which embodies the characteristic aromatic principles of the cedar wood and which, when incorporated in the plaster in the manner herein disclosed, gives to the plaster the property of emitting the characteristic aroma and fragrance of natural cedar wood unaccompanied by any sensible variant or additional odor. The term is intended to comprise any such oil, extract or essence, however obtained, which has the properties just stated.

The basic structural material of the cedar plaster of the present invention is Keene's cement. Keene's cement is a hard plaster or cement well known as a standard product in the building industry. It is made by a double burning of a pure gypsum with an intermediate chemical treatment. It constitutes a hard, smooth surfaced, durable plaster which retains its hardness throughout exceptionally long periods of time and is not subject to deterioration even under conditions where it is subject to the action of moisture, as is the case with ordinary gypsum plasters. The finished plaster of the present invention comprises a structural base of Keene's cement with the cedar wood oil ingredient incorporated with it. It is understood that other ingredients can be used as the structural base of the plaster such as, for instance, ordinary gypsum plaster or, in fact, any plaster composition or combination of plaster forming ingredients which are capable of producing a satisfactory grade of plaster and which additionally are capable of embodying the aromatic ingredient, and permitting its emission at an appropriate rate and which will not deteriorate or change the character of the aromatic ingredient. Keene's cement, however, is particularly suitable for high quality work

due to its exceptional properties as a wall surfacing material. Other cements, such as Portland cement, may be successfully used where appropriate either alone or in admixture with other suitable plaster forming ingredients or cements. A small percentage of clay may be incorporated with the Keene's cement or other base material if desired, and is of a certain advantage in making the troweling operation easier and in giving an added smoothness to the surface of the finished plaster. It has a lubricating action under the trowel, and at the same time fills in the pores of the plaster and thus aids in providing a smooth surface. The addition of an appropriate proportion of diatomaceous earth serves to somewhat increase the surface covering capacity of a given weight of the plaster. The references herein made to wall surfaces are intended to mean any walls and ceilings of rooms and buildings, floors, partitions, linings for chests and boxes, and in general any of the uses for which plaster is intended and adapted. For the purpose of increasing the adhering properties of the plaster to smooth surfaces such as old plaster walls, woods, paint, metal, etc., a small percentage of an appropriate adhesive material, for example, a combination of casein and a suitable alkaline material, such as hydrated lime to render it soluble, may be added. This is of importance particularly in adapting the plaster for use in refinishing walls of old buildings and as a lining or coating for wood or metal boxes, chests, etc. When the plaster is used for these purposes, for instance in refinishing walls of old buildings, the addition of say 3% to 5% of casein and also from say 3% to 10% of hydrated lime or Portland cement gives a coating which adheres well and does not have a tendency to deteriorate, crack or peel off. It is understood that the term plaster or plaster composition as used in the claims includes such plastic wall coating compositions as just referred to, frequently designated in the trade as plastic paints, and in general means any wall coating composition capable of application to the wall in substantial thickness in plastic state, either by trowel, by brush, or otherwise, and capable of solidifying upon the wall into a permanent solidified coating.

The active constituent of the cedar plaster of this invention, oil of cedar wood, is preferably incorporated into the plaster through the medium of an absorbent material. The absorbent material is preferably in powder, granulated, fibrous or dust form in a state of subdivision appropriately fine for incorporation into a plaster and is of such character as to absorb or take up the cedar wood oil in substantial amounts and still remain in finely divided apparently dry condition with the particles thereof separable and capable of being homogeneously admixed with the other

dry ingredients of the plaster. A satisfactory absorbent material for this purpose is wood dust, that is, finely ground wood or sawdust of appropriately fine particle size. It is understood that the wood used for this purpose does not possess any characteristic odor of its own which will objectionably modify or inhibit the natural cedar fragrance of the cedar wood oil ingredient. The cedar wood oil is thoroughly mixed with the wood dust, and the constituent particles of the dust are thus impregnated with the cedar wood oil. The wood will absorb substantial quantities of the oil and still remain in dry, powder form. The impregnated wood dust is incorporated directly with the other dry ingredients of the plaster. If desired, cedar wood dust may be used as the absorbent material and its natural aromatic value thus availed of. The percentage of the cedar wood oil in cedar wood is, however, very low so that by far the larger proportion of the cedar wood oil in the absorbent wood dust as it occurs in the plaster is derived from the impregnation of the wood dust with the oil.

25 A satisfactory cedar plaster which has been used successfully in a commercial way is constituted as follows:

|                       | Per cent |
|-----------------------|----------|
| Keene's cement        | 84       |
| 30 Cedar wood dust    | 5½       |
| Oil of cedar wood     | 6½       |
| Clay                  | 3        |
| Red coloring material | 1        |

35 The above proportions are by weight. The wood dust is mixed with the cedar wood oil until the oil has been completely absorbed in the wood dust and the particles of the dust have become thoroughly impregnated with the oil. The impregnated wood dust and the other ingredients are then mixed together to effect even distribution of the several ingredients and attain a reasonable homogeneity in the product. The above combination of ingredients constitutes a complete plaster. It is prepared for application to the wall by mixing with sufficient clean water to obtain a mixture of proper consistency for plastering. When the plaster is applied to the wall and troweled down it sets and hardens into a permanent and thoroughly high grade wall surface. The plaster is not affected by moisture, and its smooth hard surface may be washed without affecting the character of the plaster or the fragrance and aroma emitted by it. It is easy to clean and is thoroughly sanitary. The present product may be applied with the ease of ordinary plaster and is thus particularly advantageous in lining closets which are designed under the roof and in odd places. Closets, chests, containers, and the like, of any shape can readily be lined with the plaster, and when the job is finished the plaster covers the entire surface without cracks, holes or joints. The fire-proof qual-

ties of the plaster also recommend it for this work. The coloring matter is added to further carry out the simulation of true cedar. It is understood that any color design as desired may be used. The cedar plaster is preferably applied as a finished coating over an ordinary base coat of plaster. When the cedar plaster made according to the above formula is applied as a coating of about  $\frac{1}{8}$ " thick, it possesses aromatic qualities substantially equivalent to that of a lining of true cedar wood of about  $\frac{1}{8}$ " thickness. If desired, the rate of emission of the cedar aroma and the possible tendency of the cedar oil to spread into the dry plaster forming ingredients may be restricted by the use of a heavy oil such as paraffin in the manner disclosed in our copending application, Serial No. 342,296.

40 The specific formula noted above is given by way of illustration and example. The formula may be varied to suit particular conditions. For example, a satisfactory formula embodying the invention which is typical of the variations which can be made without departing from the spirit of the invention is as follows:

|                         | Per cent |
|-------------------------|----------|
| Keene's cement          | 63       |
| Sawdust of neutral odor | 5½       |
| Oil of cedar wood       | 6½       |
| Silica sand             | 25       |
| Coloring matter         | 1        |

45 The use of other absorbent materials, as for instance, asbestos, is possible, and in general any material which fulfills the requirements of an absorbent as given above and which does not carry any substantial characterizing odor of its own which will objectionably modify the true cedar aroma of the plaster.

50 The preparation of a complete plaster in dry stable powder form ready for mixing with water for application to the wall is of particular importance from a practical standpoint. Where it is necessary to ship certain ingredients of a product of this kind separately, objections such as inconvenience to the worker, difficulty of properly mixing the ingredients to a homogeneous condition on the job, lack of facilities for measuring quantities to be mixed with consequent lack of uniformity in different mixes, impossibility of getting workmen to exercise the requisite care in measuring and mixing, etc., make the proposition entirely impracticable for commercial work. This is particularly true where one of the ingredients which must be shipped separately is a liquid. The ingredients of the present plaster are sufficiently stable to resist deterioration or change during the ordinary course of manufacture, storage, shipment and use.

55 The present invention therefore provides a plaster composition which is in every sense a true plaster and which at the same time pos-

seses the property of emitting the characteristic fragrance and aroma of natural cedar wood. It brings to the user the benefits of cedar wood with the accompanying advantages of a plaster and without the disadvantages of cedar wood. The cedar plaster of this invention is defined in the following claims in terms of its novel characteristics and properties and in terms of the features of its composition and formulation which are responsible for such characteristics and properties. The term plaster as used herein designates the usual compositions of such materials as lime, gypsum, various cements, and the like, which are ordinarily referred to and classified as plasters and which are used for wall coatings and like purposes, and also includes generally any plastic or spreadable material capable of application to a wall and capable 20 of forming on the wall a finished hardened and permanent wall coating.

We claim:

1. A wall plaster composition comprising plaster forming material and odor emitting material of such a character and in such amount as to emit the characterizing and predominating aroma of cedar wood from the solidified plaster after application and solidification upon the wall.
2. A wall coating, substantially as described, which comprises plaster forming material in solidified condition upon the wall and odor emitting material incorporated therein of such a character and in such amount as to emit the characterizing and predominating aroma of cedar wood.
3. A wall plaster composition of the character disclosed, which comprises plaster forming material, aromatic cedar matter in such amount as to emit the characterizing and predominating true aroma of cedar wood from the solidified plaster after application and solidification upon the wall, and a heavy oil for restricting the rate of aroma emission.
4. A wall plaster composition comprising plaster forming material and aromatic cedar matter effecting emission of a characterizing and predominating true aroma of cedar from the solidified plaster after application and solidification upon the wall and, in combination therewith, paraffin, whereby said plaster composition is characterized by substantial permanence of aroma emission.
5. A wall coating composition which comprises spreadable plastic material including casein in the presence of alkaline matter and aromatic cedar matter effecting emission of a characterizing and predominating true aroma of cedar from the solidified wall coating after application and solidification upon the wall.
6. A wall plaster composition comprising plaster forming material and, in combination therewith, volatile aromatic cedar matter present in proportion by weight at least

equal to the proportion of volatile aromatic oil normally present in genuine cedar wood, effecting prolonged emission of a characterizing and predominating readily perceptible aroma of cedar from the solidified plaster after application and solidification upon the wall.

7. As an article of manufacture, a wall plaster composition of the character disclosed which comprises, in combination and in ~~dry~~ <sup>75</sup> homogeneous physical admixture, plaster forming material substantially free from odor yielding principle, and a separate absorbent vehicle independently impregnated with active volatile aromatic cedar matter present in said absorbent vehicle in proportion substantially in excess of the proportion of cedar wood oil in genuine cedar wood, effecting slow prolonged emission of a characterizing and predominating readily perceptible true aroma of cedar from the solidified plaster after application and solidification upon the wall.

In testimony whereof we affix our signatures.

EDWIN D. CODDINGTON.  
ERNEST A. KERLER.  
ROE R. BLACK.  
HARVEY S. OWEN.

90

95

100

105

110

115

120

125

130